

March 13, 1934.

S. RUBEN

1,950,750

RESISTANCE DEVICE

Filed Feb. 3, 1931

FIG.1.



FIG.2.



FIG.3.



INVENTOR  
SAMUEL RUBEN

BY HIS ATTORNEY *MacCay & Lamm*

## UNITED STATES PATENT OFFICE

1,950,750

## RESISTANCE DEVICE

Samuel Ruben, New Rochelle, N. Y., assignor to  
 Ruben Patents Company, New Rochelle, N. Y.,  
 a corporation of Delaware

Application February 3, 1931, Serial No. 513,083

6 Claims. (Cl. 201—55)

This invention relates to a resistance device and to the method of making it. An object of the invention is the provision of a resistance device capable of withstanding the effects of over-5 loads and unfavorable atmospheric conditions and which lends itself to accurate duplication in commercial production.

This invention constitutes an improvement upon my co-pending applications filed September 17, 1928, and October 6, 1930, bearing respectively Serial Numbers 306,608, and 486,698. These issued as Patents 1,877,482 and 1,859,344 on Sept. 13, 1932 and May 24, 1932 respectively.

The resistance element of this invention consists of a base of a compound of high specific resistance, such as copper oxide and having a coating closely adherent to the surface of the base consisting of a deflocculated graphite, the element itself consisting preferably of an arcuate 20 plate. The method of securing the surface coating is to suspend the heated base plate in a concentrated solution of ammonia in which colloidal graphite is in suspension. There is then deposited on the copper oxide plate a layer of 25 graphite and cuprous amino-oxide; the coated plate is then raised to a temperature at which the ammonia is volatilized and a hard coating of deflocculated graphite firmly adheres to the compound base. One advantage of this treatment 30 lies in the uniform thickness of the resistance coating, or graphite layer.

A suitable movable contact may be provided for a variable resistance device. Otherwise, the two contact members may remain stationary. 35 By varying the thickness of the graphite coating, the degree of resistance offered by the element may be fixed.

Reference to the accompanying drawing will assist in understanding the invention. In the 40 drawing Fig. 1 diagrammatically shows a plan view of the device, Fig. 2 a cross section at 2—2 and Fig. 3 a cross section of the resistance element.

In the drawing 1 represents the cuprous oxide 45 graphite coated resistance element, 2 the insulator base to which it is attached and 3 and 4 the terminals of the resistance plate. At 5 is an arm rotatable on shaft 7 and carrying contact plate 6, in contact with the resistance plate 1. At 9 is 50 a head attached to shaft 7 for rotating the arm 5, 10 being a nut lock and 11 representing compression springs to insure uniform contact between contact bar 6 and resistance plate 1.

Fig. 3 shows the arch construction of resistance element 1.

For general use the most satisfactory base material is cuprous oxide; however, other materials such as iron oxides and other conductive oxides, sulphides, selenides and tellurides can be used for this purpose.

In the production of the resistance element controlling factors are the graphite content in the ammonia mixture and the temperature to which the coated element is heated. It has been found that by heating the coated plate to between 65 35° and 400° C. its resistance is about one-thirtieth of that prior to the application of heat. It has also been determined that if the temperature is raised beyond about 400° C. the resistance of the element increases materially. Thus for 70 lower resistance the element should be heated to between 350° and 400° C. which permits the use of a minimum thickness of graphite coating. Measuring one sample of this device it is found that without the application of heat it had a 75 resistance of about 15,000 ohms after being dipped in a solution containing 5% of solid graphite; but after heating to 350° C. the resistance dropped to 500 ohms.

In the heating process a cuprous amino-oxide 80 is formed by the reaction of the strong ammonia with the cuprous oxide surface. This compound is very effective as a binder, causing a strong adherence between the hard graphite layer and the surface of the base element.

## What I claim is:

1. A resistance element comprising a base of a crystalline compound of the class comprising the electronically conductive oxides, sulphides, selenides, and tellurides, having a lower resistance surface comprising the reaction product of an ammonia-graphite mixture with the base material.

2. A resistance element comprising a base of a crystalline compound of the class comprising 95 the electronically conductive oxides, sulphides, selenides, and tellurides, having a lower resistance surface comprising the reaction product of an ammonia-graphite mixture heated with the base material.

3. A variable resistance element comprising a base of a crystalline compound of the class comprising the electronically conductive oxides, sulphides, selenides, and tellurides, having a lower 105 resistance surface comprising the reaction product of an ammonia-graphite mixture with the base material.

4. A variable resistance element comprising a base composed of an electronically conductive oxide and having a lower resistance surface com- 110

prising the reaction product of an ammonia-graphite mixture with the base material.

5. A variable resistance element comprising a base composed of copper oxide having a lower 5 resistance surface comprising the reaction product of an ammonia-graphite mixture with the base material.

6. The method of making a resistance element which consists in coating a base plate composed of copper oxide with a solution of ammonia in which colloidal graphite is suspended, heating said plate until the ammonia graphite mixture 80 combines with the copper oxide.

SAMUEL RUBEN.

10

85

15

90

20

95

25

100

30

105

35

110

40

115

45

120

50

125

55

130

60

135

65

140

70

145

75

150